

Patented Sept. 29, 1925.

1,555,315

# UNITED STATES PATENT OFFICE.

WILHELM ROHN, OF HANAU, GERMANY.

PIN FOR ARTIFICIAL TEETH, SMALL RINGS, FUSING-IN WIRES, AND THE LIKE.

No Drawing.

Application filed April 13, 1920. Serial No. 373,606.

(GRANTED UNDER THE PROVISIONS OF THE ACT OF MARCH 3, 1921, 41 STAT. L., 1313.)

To all whom it may concern:

Be it known that I, WILHELM ROHN, a citizen of Germany, and resident of Hanau, Germany, have invented new and useful 5 Pins for Artificial Teeth, Small Rings, Fusing-in Wires, and the like (for which I filed an application in Germany, April 18, 1918, now Patent No. 348,917), of which the following is a specification.

10 Technically produced metals contain, as is well known, considerable quantities of gases in solution. It is further known that such metals will, under favorable conditions, yield up the whole or a part of their content of gas. This is particularly disagreeable when wires drawn of such metals or alloys are fused into ceramic or glassy materials, as this is, for example, necessary with the fusing-in wires conducting the current to the incandescent wire for electric incandescent lamps or Röntgen-ray tubes or the like, or also in fusing the pins into the porcelain body of artificial teeth. When leading-in wires are fused into glass they 15 will, frequently, even if the coefficient of heat-expansion of the wire is absolutely the same as that of the glass, be surrounded by a whole coat of vesicles enclosing the surface of the wire fused into the glass. According to the fusing-in process employed this coat or vesicles may consist of a few large bubbles or of a vast number of extremely fine bubbles. It is obvious that this 20 is not favorable for the quality, the reliability and the hermetical quality of the fusing-in. The same is the case with artificial teeth. If such an artificial tooth is broken apart at the place where the pin, say of technical nickel, has been fused into it, one will frequently find one or more, comparatively large air bubbles, which greatly impair the strength of the joint between tooth and pin; frequently these bubbles will even be so large that the outer form of the 25 tooth suffers in consequence by being bulged out. Even encased wires, consisting of a core wire of say technical nickel or some other metal or alloy with a covering of precious metal such as gold or platinum rolled on, will show the same annoying phenomenon wherever this casing is in any respect unsound, for example at the point of the pin or at cut surfaces.

30 Applicant has described in a separate

United States application Serial Number 363,916, filed March 6, 1920, processes invented by himself, by means of which a sufficient degasification of metals and metal alloys may be obtained by keeping such metals or metal alloys molten for some time under a constant but low pressure, or by frequently remelting them under the said conditions. In this before-mentioned pending application, before degasifying the metals, by melting them under reduced pressure in a practically absolutely airtight melting furnace, it is necessary in so far as their properties when in molten state are not fully known, to ascertain by experiment, at which temperatures gases are generated, and at which temperatures dissolved gases are expelled. These temperatures being ascertained, the respective metal can be obtained continuously with the same good qualities by treating it at the said temperatures. For example, an alloy of nickel and chromium which had been melted according to the process forming the subject-matter of the invention at a pressure of 1 mm. mercury column and 1440° C., after previously showing a liberal evolution of gas, remains quite calm and apparently free of gases. When subsequently worked, the metal showed bad qualities and tended to crack. The same alloy being then melted at varying pressures and temperatures, it was found that at a pressure of 3 mm. mercury column and a temperature of 1460° C., a second very violent emission of gas occurred. The product of this melt was, on being worked, found to be perfect. All the numerous alloys of the same composition melted since that time were melted at 1460° C. and 1-3 mm. mercury column pressure. They all had a second emission of gas and subsequently showed all the same unexpectedly good qualities.

35 In all cases in which gases are emitted or produced during the solidification the metal bath must first be cooled down to a temperature, at which the said gases are emitted. Thereupon the metal should be re-melted and the gases liberated be drawn off. With a few metals and alloys it is necessary to repeat such re-melting. With iron, for instance, a repeated melting may be necessary in all those cases, in which the perfect chemical equilibrium between all components

55

60

70

75

80

85

90

95

100

105

both in liquid as well as also particularly is viscous and in solid state not yet had been attained after the first melting.

- For example, an alloy of iron and cobalt 5 will appear free of gas in the molten state; neither an increase of temperature nor a reduction of the pressure will be able to cause a further emission of gas. Only when solidification sets in, a lively emission of gas 10 commences and will continue until the alloy is fully solidified. An immediate re-melting will show neither a further emission of gas during the melting nor from the molten metal, but only will allow the escape of the 15 mechanically included gases of the first melting. A renewed solidification liberates no more gas, and the product shows in every respect freedom of gas flawless and good properties.
- 20 Extensive tests have shown that such metals remain free from gases, when they are subsequently worked or annealed in presence of various gases and under various pressures. It has, in fact, been found, that 25 in fusing-in thin plates, sheets, rings, wires or the like, made of such metals or metal

alloys, the fused joint remains fully free from bubbles, which certainly means an important improvement in practice.

When the wires consist of a base metal 30 core with a rolled on casing of precious metal, the said core is freed from gas in the same manner. With the precious metals employed as casing, viz platinum and gold, this removal of gas is unnecessary as these metals 35 as a rule do not contain any gases in solution, except of course if they are of insufficient purity.

What I claim is:

A ceramic metal joint comprising a fine 40 metal part composed of metal rendered substantially free from gas by successively remelting in a substantially airtight furnace at different predetermined values of temperature and reduced pressure, and a 45 ceramic mass plastically closed around said part while hot.

In testimony, that I claim the foregoing as my invention I have signed my name this 27 day of February 1920.

DR. WILHELM ROHN.